

## UNITED STATES PATENT OFFICE.

EXAMINER

et al

WILLIAM N. HAAS AND HERBERT C. YOUNG, OF DENVER, COLORADO, ASSIGNORS, BY  
DIRECT AND MESNE ASSIGNMENTS, TO ROKO MFG. CO., OF DENVER, COLORADO, A  
CORPORATION OF COLORADO.

1,273,361

## COMPOSITION FOR USE WITH PRINTERS' INK.

1,273,361.

Specification of Letters Patent. Patented July 23, 1918.

No Drawing. Application filed October 5, 1916, Serial No. 123,947. Renewed January 29, 1918. Serial No. 214,416.

106-316

To all whom it may concern:

Be it known that we, WILLIAM N. HAAS, and HERBERT C. YOUNG, citizens of the United States, residing at Denver, in the county of Denver and State of Colorado, have invented new and useful Improvements in Composition for Use with Printers' Ink, of which the following is a specification.

This invention relates to a composition for use with printers' and lithographers' inks for the purpose of overcoming certain objections incident to the use of ordinary inks of various kinds, grades and colors and at the same time imparting desirable and valuable properties thereto.

The primary object of the invention is to provide a composition which, when mixed with printers' ink, will serve as a reducer and spreader to increase the covering capacity of the ink, as an intensifier to promote and increase the color tone or effect and impart a finer degree of appearance to high, medium and low grade inks, and to secure rapid setting qualities, whereby the printed stock may be quickly handled and stacked without offsetting and similar objections.

A further object of the invention is to provide a composition of the character described which insures economy in the use of ink, which provides for the more even and uniform distribution of the ink to the surfaces of the form and surfaces being printed, which eliminates sticking, blank spots, picking, and the greasy and mottling effects produced by some inks, and which prevents or reduces electrical manifestations ordinarily set up in the process of printing.

A still further object of the invention is to provide a composition of the character described which will, without destroying the working condition of ink while on press, quickly set the ink on non-absorbent, enameled, glazed or similar surfaces with sufficient rapidity to permit of the stacking of the printed sheets to any degree as fast as impressions are taken without offsetting, thus avoiding slip-sheeting and other expensive measures generally taken for preventing blurring, offsetting and like difficulties in the employment of printers' inks in common use.

In carrying our invention into practice,

Comptac  
for 1000

we provide a composition of the character and for the purpose set forth consisting of an intimate admixture or combination of petrolatum, magnesium carbonate, and sodium silicate, in the proportions of one pound of petrolatum to from two to three ounces of magnesium carbonate, and from one-fourth to one full fluid ounce of sodium silicate, a mixture of the ingredients in the proportions of one pound of petrolatum to 2.5 ounces of the magnesium carbonate and one-half fluid ounce of the sodium silicate being preferred as best adapted for ordinary or general use.

In combining the ingredients to produce the composition, the petrolatum and magnesium carbonate are first thoroughly combined and mixed together, and then the sodium silicate is added and mixed thoroughly therewith, any suitable form of agitating or mixing device being employed.

In the use of the composition, one part of the composition is mixed with from four to five parts of the ink, but a greater or less amount of the composition may be employed according to the character and grade of ink. If an excessive proportion of the composition is used, it will not dry upon press or otherwise affect its working condition. As the better grades of ink carry a larger proportion of pigment, such inks will stand a greater reduction than the lower grades. The ink thus combined with the composition is then employed in any of the ordinary ways for printing or lithographing purposes. It is to be understood, of course, that the amount of the composition used in connection with any certain amount of ink may be varied to some considerable degree, dependent upon the particular character of the ink, the nature or character of the work to be done and climatic or other conditions.

In this composition, the petrolatum is employed as a base having qualities to adapt it to intimately combine with printers' and lithographers' inks. As this substance has a greasy effect, the magnesium is added thereto to neutralize such effect, resulting in a mixture that will release itself readily without pull and practically in its entirety from surfaces used for producing printed impressions, such as wooden or metallic printing type, zinc etchings, half-tone etch-

ings, etc. The magnesium further serves as a drying agent, but possesses the objection of not adhering well to paper.

The sodium silicate is employed in the composition as a binder for the ingredients in combination with the ink, and as both an adhesive and a drying agent, the sodium silicate, being distributed throughout the mass, overcoming the non-sticking properties of the magnesium carbonate and causing all the particles of the mass to adhere to each other and to paper and other surfaces. In this composition, the magnesium carbonate neutralizes the oiliness of the petrolatum, while the sodium silicate in addition to supplying adhesive and drying properties further performs the functions of a tone intensifying producing agent.

In printing upon paper with an ink with which the composition is combined, the air coming in contact with the surface of the ink between impressions causes the sodium silicate to harden and the ink surface to set in a practically instantaneous manner, forming a film that protects the impression under ordinary handling against blurring or destruction by the next printed article delivered upon it, until such time as it is thoroughly set. In practice, it is found that the surface of the ink sets with sufficient rapidity to permit of the stacking of the stock to any height as fast as it comes from the press, without offsetting, thus eliminating slip-sheeting and stacking in trays in small quantities and saving labor required for slip-sheeting. This result is obtained in the printing of various kinds of papers, including hard non-absorbent papers such as enameled, ledger or bond papers, and, owing to the rapidity of the setting action, subsequent impressions may be taken, ink on ink, or backing up performed on enameled, bond or ledger papers within a considerably shorter period than could be done with original ink without offsetting.

It is understood, of course, that the composition, when mixed with ink, tends to lessen the proportionate amount of coloring matter, but the composition has an intensifying action in increasing the color tones, and when used within certain limitations produces a color effect in excess of that of the original ink. It may be used to equal advantage in black, white or any color of ink in proportion to the result or effect most desired.

In the process of taking a printed impression in using an ink with the composition mixed therewith no sticking or tacking occurs, practically all of the ink being released readily on the object printed upon. The ink also lies flat, eliminating blank

spots, picking, crawls and other imperfections or objections, so that a smooth unbroken distribution of ink is obtained on the surface of the object printed. The composition when used with news ink will enable this and other oily kinds of ink to be used upon hard-surfaced or non-absorbent paper, will increase the fineness of texture and covering properties of all kinds and grades of ink, and also improve the color tone of the ink and impart a fine finish to even low grade inks. The composition is not affected to any material extent by climatic conditions and imparts its properties in this respect to the ink, enabling the ink to be worked freely at low temperatures and thus overcoming difficulties experienced in printing establishments when the temperature falls below a certain degree. As the composition increases the setting quality of the ink, a larger supply of ink may be fed from a supply fount or carried upon an inking plate than is possible in the use of plain inks, resulting in a heavy full-tone impression.

An important feature incident to the use of the composition is that it serves as an electrical insulator by means of which the generation of static electricity during the process of printing is entirely or practically eliminated, thus overcoming all the difficulties experienced in handling electrically loaded paper. Inasmuch as the composition may be used without strict regard to proportions within certain limits, the composition may be mixed with ink and the treated ink used by unskilled hands or apprentices. The composition may be used with all kinds of inks, including double-tone, with the exception of copying inks.

Having thus described our invention, we claim:

1. A composition for use with printers' ink embodying a mixture of petrolatum, magnesium carbonate, and sodium silicate.

2. A composition for use with printers' ink embodying a mixture of petrolatum, about one pound, magnesium carbonate, from two to three ounces, and sodium silicate from one-fourth to one full fluid ounce.

3. A composition for use with printers' ink embodying a mixture of petrolatum, one pound, magnesium carbonate, 2.5 ounces, and sodium silicate one-fourth fluid ounce.

In testimony whereof we affix our signatures in presence of two witnesses.

WITNESSES: WILLIAM N. HAAS.  
HERBERT C. YOUNG.

Witnesses: ELSIE WEBER,  
R. E. KRAMER,